

# UNITED STATES PATENT OFFICE.

EDWARD KELLER, OF BALTIMORE, MARYLAND.

## METHOD OF MAKING ALLOYS.

SPECIFICATION forming part of Letters Patent No. 696,244, dated March 25, 1902.

Application filed November 15, 1899. Serial No. 737,055. (No specimens.)

*To all whom it may concern:*

Be it known that I, EDWARD KELLER, a citizen of the United States, and a resident of Baltimore, in the State of Maryland, have 5 discovered certain new and useful Improvements in the Method of Preventing and Reducing Concentration and Dispersion of Impurities as Consequent Effect of Segregation in Alloys; and I do hereby declare the following to be a full, clear, and exact description of the same.

In the melting and casting of metal it has been discovered by a long course of experimentation and observation that foreign metals, metalloids, &c., held in solution in the solvent metal tend as the metal freezes or solidifies to accumulate or predominate at certain centers or zones. This tendency is entirely independent of any gravity separation 20 occurring while the mass is in its molten or liquid condition and results in a casting the several parts of which vary in the relative proportions of their constituent elements. This unequal distribution of the elements of 25 a casting has been termed "segregation," which term I shall adopt herein, and it is obvious that as a result of it castings designed for strength are liable to be weak in certain portions without the possibility of detection 30 until the weakness is developed by fracture. So, too, should the casting—an ingot, for instance—be designed for assaying, samples taken from any one portion will not give a true indication of the relative proportions of 35 the metals in the entire mass, but may assay either above or below the average, depending upon whether the impurities have accumulated or not at the particular point where the sample is taken. The metal, metalloids, &c., 40 which occasion the phenomenon of segregation I shall herein term "impurities," although any one or more of them may be valuable, if not the most valuable constituent or constituents of the mass, even though existing in 45 relatively small quantities.

In the most prominent and general form of segregation the impurities tend toward the portions of the metal last to solidify, while in other forms of segregation the opposite effect

is observed—*i. e.*, the impurities tend toward 50 those portions of the mass the first to solidify. In either case the tendency to segregate may result in a series of zones having varying proportions of the constituent elements of the mass.

I have discovered that segregation may be greatly reduced by combining the solvent metal and impurities in such proportions that the solvent metal will be saturated with the impurities when at the freezing or solidifying 60 temperature. In other words, I have observed that metals at freezing or solidifying temperature have a certain capacity for holding in solution a given quantity of impurities without tending to segregate. Subsaturation I 65 have discovered causes a segregation toward the center of solidification and supersaturation causes a segregation in the opposite direction.

Each metal, metalloid, &c., has a definite 70 point of saturation in every solvent metal. The point of saturation becomes variable when more than one element is dissolved. Thus the saturation-points for a number of elements are interdependent. From this it 75 follows that the saturation-point of one element is lowered by the solution of one or more other elements, and when the solvent is subsaturated with one element or with a number of elements and segregation toward the center of solidification takes place the addition of the same element or of other elements in quantity sufficient to charge the solvent to the saturation-point at solidifying temperature will retard, reduce, or prevent segregation. 80 85

In case of segregation toward the portions of the mass first to solidify because of supersaturation some of the impurities must be eliminated or additional purer solvent metal 90 added to give a saturated solution at the freezing temperature.

The addition to be made to the mass to bring it to the saturation-point at the freezing temperature must be determined empirically—for instance, by analysis of samples taken from certain portions of sample castings, which when they show segregation and

the degree of segregation toward the center of solidification indicate subsaturation and the quantity of impurity to be added to bring the mass up to the point of saturation.

- 5 Obviously in the practical application of my discovery experience in handling metals of a certain grade where segregation occurs will enable the operator to add an impurity in the first instance without sampling, which 10 will benefit the solvent metal in its industrial application and at the same time reduce or prevent segregation due to the impurities which already exist and cannot be entirely eliminated or which have been added to produce a desired alloy or combination of metals.

15 Many practical examples wherein segregation has been greatly lessened or prevented for all practical purposes might be given; but the following will answer for illustrative purposes, viz: Refined copper was the metal employed, and from a batch of this metal a block was cast of convenient size rectangular in shape and samples were taken vertically and approximately through the center of solidification or last portion of the mass to solidify. The analysis was made of each inch in vertical height, starting at the top, and the following tables are based on the percentage of two impurities—silver and gold—per ton.

20 Thus:

|    |                   | Ag oz.<br>per<br>ton. | Au oz.<br>per<br>ton. |
|----|-------------------|-----------------------|-----------------------|
| 35 | First inch .....  | 85.67                 | 0.28                  |
|    | 1/3 inch .....    | 88.15                 |                       |
|    | 2/3 inch .....    | 89.5                  | 0.24                  |
|    | Third inch .....  | 87.0                  | 0.24                  |
|    | Fourth inch ..... | 86.1                  | 0.26                  |
|    | Fifth inch .....  | 84.6                  | 0.23                  |

- 40 This shows a segregation toward the center of solidification, which is a point near the vertical center and toward the top of the mass. By adding a small quantity of lead analysis 45 showed the following results:

|    |                   | Ag oz.<br>per<br>ton. | Au oz.<br>per<br>ton. |
|----|-------------------|-----------------------|-----------------------|
| 50 | First inch .....  | 86.0                  | 0.22                  |
|    | Second inch ..... | 85.8                  | 0.24                  |
|    | Third inch .....  | 85.3                  | 0.24                  |
|    | Fourth inch ..... | 86.2                  | 0.24                  |
|    | Fifth inch .....  | 85.7                  | 0.22                  |

- 55 By adding zinc the following results were obtained:

|    |                   | Ag oz.<br>per<br>ton. | Au oz.<br>per<br>ton. |
|----|-------------------|-----------------------|-----------------------|
| 60 | First inch .....  | 85.0                  | 0.28                  |
|    | Second inch ..... | 84.0                  | 0.26                  |
|    | Third inch .....  | 86.6                  | 0.28                  |
|    | Fourth inch ..... | 85.0                  | 0.28                  |
|    | Fifth inch .....  | 86.1                  | 0.28                  |

By adding nickel the following results were 65 obtained:

|                   | Nickel.<br>Per ct. | Ag oz.<br>per<br>ton. | Au oz.<br>per<br>ton. |
|-------------------|--------------------|-----------------------|-----------------------|
| First inch .....  | 0.40               | 88.0                  | 0.26                  |
| Second inch ..... | 0.36               | 87.1                  | 0.24                  |
| Third inch .....  | 0.38               | 85.5                  | 0.26                  |
| Fourth inch ..... | 0.35               | 87.8                  | 0.28                  |
| Fifth inch .....  | 0.36               | 87.6                  | 0.22                  |

70

75

The same grade of copper as the above refined copper when containing a small amount of sulfur becomes what is known as "blister copper," which shows segregation to a much more marked degree, yet on adding more sulfur this segregation may be reduced or even prevented, as shown by the following illustrations:

20 A copper containing about 0.5 per cent. of sulfur shows the following segregation for silver and gold:

|                   | Ag oz.<br>per<br>ton. | Au oz.<br>per<br>ton. |
|-------------------|-----------------------|-----------------------|
| First inch .....  | 99.2                  | 0.26                  |
| Second inch ..... | 98.1                  | 0.26                  |
| Third inch .....  | 102.3                 | 0.28                  |
| Fourth inch ..... | 77.4                  | 0.26                  |
| Fifth inch .....  | 78.3                  | 0.26                  |

95

On increasing the tenor of sulfur to about 0.9 per cent. the segregation is shown to be reduced as follows:

|                   | Ag oz.<br>per<br>ton. | Au oz.<br>per<br>ton. |
|-------------------|-----------------------|-----------------------|
| First inch .....  | 80.2                  | 0.20                  |
| Second inch ..... | 84.5                  | 0.24                  |
| Third inch .....  | 87.8                  | 0.22                  |
| Fourth inch ..... | 88.3                  | 0.24                  |
| Fifth inch .....  | 87.4                  | 0.26                  |

100

105

110 It appears, therefore, that by adding a small quantity of an impurity to the solvent metal when segregation toward the center of solidification occurs the tendency to segregate in this direction is lessened and uniformity of the mass greatly increased. The amount to be added, as before stated, must be determined empirically inasmuch as it will vary with the aggregate impurities contained in the solvent metal.

115 Having thus described my discovery, what I claim is—

1. The method of reducing segregation in cast metal, which consists, first, in determining by analysis of a casting, whether segregation occurs toward or away from those portions of the casting first to solidify, and secondly in combining with the remelted metal or other portion of the same batch of metal when in a fluid condition, a substance for

120

115

125

eign thereto, but soluble therein in such quantity as to maintain a homogeneity of the mass at the solidifying or freezing temperature and finally casting the treated molten metal; substantially as described.

2. The method of reducing segregation in cast metal containing a basic metal and a material foreign thereto but soluble therein, which consists first in ascertaining whether segregation occurs toward or away from those portions of the casting first to solidify,

secondly in varying the proportion of foreign soluble material in the mass in accordance with the previously ascertained direction and degree of segregation to maintain a homogeneity of the mass at the solidifying or freezing temperature and finally casting the treated molten metal; substantially as described.

EDWARD KELLER.

Witnesses:

JOHN JOHNS,

THOMAS J. RIGNEY.